

Patented Mar. 8, 1938

2,110,383

# UNITED STATES PATENT OFFICE

2,110,383

## PROCESS FOR RENDERING WOOL TEXTILES REPELLENT TO WATER AND PRODUCT MADE THEREBY

Alexander Nathansohn, Berlin, Germany, as-  
signor to the firm Studiengesellschaft für  
Faserveredelung m. b. H., Berlin, Germany

No Drawing. Application November 10, 1934, Se-  
rial No. 752,532. In Germany December 4, 1933

### 7. Claims.

(Cl. 68—37)

The present invention relates to improvements in or relating to the treatment of wool textiles for the purpose of rendering such textiles repellent to water.

5 Various processes have already been proposed for rendering wool repellent to water. Generally these processes may be divided into three groups as follows:—

(1) Processes in which emulsions of paraffin 10 or the like are used;

(2) Processes in which aluminium compounds are used;

(3) Processes in which the wool is treated 15 with anhydrides of higher fatty acids.

15 All these processes have the disadvantage that they do not always meet the maximum of requirements. The processes under (1) produce good effects, but the latter are not always sufficiently stable towards washing with soap. Further when

20 such processes are used on fine knitted goods the quality of the latter is affected. The processes according to (2) yield in part products which also do not well resist washing with soap or, if the products are greatly resistant to washing the

25 processes, give them a hard feel. In the processes under (3), in which raised temperatures have to be used, trouble may be caused by the yellow dis- coloration of the wool which may occur in cer- tain cases. Moreover this process can only be 30 carried out in installations which have the spe- cial equipment that is required for that purpose.

The process described below is characterized by the fact that it yields products of non-de- 35 teriorated quality and that the effects obtained with such process have in practice an unlimited resistance towards the usual washing agents.

The process is based on the surprising discovery that wool is rendered to a high degree repellent to water in every stage of the working up pro- 40 cesses, that is to say as loose wool, yarn, fabric and in the form of knitted and woven goods whether in a raw, bleached or dyed condition, by treatment with solutions of water-soluble salts of higher fatty acids, that is to say, acids with at 45 least 10 carbon atoms, provided this treatment is carried out after the goods have been thoroughly cleaned. It is an essential condition of this surprising effect, which has not hitherto been ob- 50 served, that the surface of the fibres must be freed of impurities.

55 After the treatment, the goods have to be rinsed, preferably in cold water. For rinsing, water of condensation may be used, or softened water or ordinary water as used in operating a textile works. If the water for operating the

textile works is particularly hard it may be advantageous to perform the rinsing in known manner with the use of suitable softening agents.

The following examples may serve to illustrate the process of the invention.

1. Combed wool yarn, dyed from an acid bath, is very carefully rinsed by agitating in water immediately after the dyeing operation or after it has been dried. If the rinsing liquor becomes acid there is added, if desired after replacing the 10 water several times, sufficient ammonia, soda or other substance of alkaline reaction until the liquor has become quite neutral. The yarn is then treated—with or without previous drying—with 20 times its weight of an aqueous solution 15 containing 3 grams of shredded commercial pot- ash soap and 0.3 gram of calcined sodium car- bonate per litre while agitating for 20 minutes at a temperature of 25–30° C. The yarn is then rinsed well (until it has become practically odor- 20 less) and is dried. The yarn is found to be re- repellent to water to a high degree.

2. Fulled cloth, which has been dyed in the piece from an acid bath, is first cleaned in the same way as the yarn in Example 1 and is then 25 treated for 10 minutes and at a temperature of 35° C. in a washing machine with 20 times the quantity of a liquor consisting of an aqueous solution of 5 grams coconut-fat potassium soap with frequent squeezing off. The material is first 30 rinsed with condenser water, then with hard water to which about 0.15 gram of a softening agent containing Turkey red oil was added, and finally the material was washed again for a short time with condenser water. After drying the cloth is 35 roughened, brushed, shorn and hot-pressed. The cloth has become remarkably resistant to water.

3. Field-gray cloth for uniforms, made from dyed loose wool, is carefully washed and neu- tralized after it has been fulled and carbonized. 40 In order to clean the cloth completely, it is treated with a solution of 0.2 gram of a syn- synthetic washing agent, such as Turkey red oil or preparations made up from sulphonated higher fatty alcohols, per litre and is well rinsed; it is 45 then treated in a washing machine for 25 minutes at a temperature of 25–27° C. with a solution as described in Example 1 or 2. The material is finished in the usual manner and has the same 50 strong water repelling capacity as that of Ex- ample 2.

4. Gabardine, dyed from an acid bath, is washed in a bath containing 0.2 gram of a syn- synthetic washing agent per litre with addition of so much ammonia that the liquor remains neu- 55

tral even after prolonged treatment of the cloth. It is then rinsed and subjected to the usual mechanical finishing process. The material is eminently suitable for making rain-coats.

5 The usual textile soaps, such for example as the shredded potash soaps used for fulling or the like, may be used for the process according to the invention; but it has been found to be advantageous to use such soaps as do not have an 10 unpleasant smell. Not only is it relatively difficult to remove such a smell from the goods, but moreover some of odoriferous substances, especially those of an aldehyde nature, are detrimental to the creation of the effect, as they are 15 strongly adsorbed by the fibre and consequently act as a harmful impurity. It is therefore advisable to produce the soap to be used in the process from fats or fatty acids which have been de-odorized in the usual manner.

20 Woolen goods of any kind may be treated in the same manner. The various kinds of water-soluble salts of higher fatty acids, such as potassium and sodium salts of saturated and unsaturated fatty acids or mixtures thereof, may be 25 used for the purpose. Commercial soaps such as the shredded potash soaps already referred to, Marseilles soap, soap flakes and soap powder may be used. The concentration may be varied but, in order to obtain good results, not less than 0.5 30 gram per litre and for practical purposes not more than 10 grams per litre are used. If the concentration is too high, the process becomes uneconomical and inferior results are produced. It is usual therefore to use from 1 to 4 grams 35 per litre. The temperatures are held preferably between 25 and 30° C.; in the case of thicker materials it may be advantageous to raise the temperature to 40-50° C. The duration of the process has a comparatively small influence on the 40 effect when the temperatures are low; it seems to be produced almost instantaneously and it is immaterial whether the treatment lasts for 5 minutes, 10 minutes, 30 minutes or an hour. At higher temperatures the effect deteriorates if the 45 treatment is prolonged; for instance at 50° the treatment is not continued for more than 1/4 hour.

It is seen from these examples that it is advisable to work at temperatures of at least 25° C.

50 The addition of sodium carbonate or its equivalents is always advantageous if there is a possibility of the material still containing traces of acid, but the addition of sodium carbonate may be useful also in other cases; it is not however 55 used in quantities larger than 2 grams per litre.

It is sometimes advisable when a sufficient resistance to water is not obtained by a single treatment according to the process of the invention, to repeat the process once or twice on the same 60 material.

It will appear from the above observations that the process can be carried out successfully in very different ways provided that the main condition, that is to say, the cleanliness of the material to be 65 treated, is fulfilled. The mode of carrying out the process thus depends to a large extent on the pretreatment to which the material was subjected and on whether impurities due to the pretreatment and which can only with difficulty be washed 70 out, adhere to the fibres or not. The process can most easily be carried out with success on materials which have previously been dyed in the boiling liquor of an acid bath. This dyeing operation involves in itself a thorough cleaning of the fibre and if the cleaning is merely completed by

very careful rinsing and neutralization, the treatment produces the most favorable results without further difficulty. Greater attention is necessary however if the material has finally been fulled or subjected to carbonization. In such cases the 5 ordinary rinsing is frequently insufficient in order to free the fibre from substances which are active on the surface. In such cases it is necessary in order, for reasons of economy, to avoid a repeated treatment of the material, to carry out the preliminary washing with particular care, either by using soap in higher concentration and in a short liquor or by using synthetic washing agents or alumina. The preliminary washing is always accompanied by neutralization. 15

The quantity of liquor which is used for the actual treatment depends in some measure on the pretreatment of the material. In the case of materials such as the last mentioned goods, or bleached goods, where small quantities of products of decomposition may adhere to the fibre despite careful preliminary washing, the liquor must in no case be too short, and in such cases the treatment is generally carried out with 10-20 times the quantity of liquid, so that the accumulation in the liquor of any decomposition products which may still be present does not attain too high a concentration. In other cases, for instance when the goods have been dyed from an acid bath, the liquor can generally be reduced 20 without disadvantage. In order to have a safe margin the treatment is not usually carried out with liquor in quantity less than 5 to 10 times the weight of the material to be treated. 25

As the effect is destroyed by acid, the new impregnation must always be carried out after the last acid treatment, that is to say after dyeing and after carbonizing. The fulling and bleaching should also preferably precede it. However all the finishing processes which are carried out 30 by mechanical means or steam may follow the impregnating process. 35

The requirement that the treatment with salts of higher fatty acids according to the invention must be carried out on material that 40 has been cleaned, explains the fact that the observation which underlies the present invention has not hitherto been made. The treatment with soap and sodium carbonate in cloth manufacture or in the working up of wool as combed wool or 45 yarns has been carried out mainly for the purpose of removing grease from such material, or in some cases for the purpose of removing fatty substances with which such goods become contaminated during their process of manufacture. 50 Cloth is subjected in such cases to a very intensive treatment with soap and sodium carbonate, for instance a piece of cloth of 30 kilograms dry weight is treated with 30 litres of soda lye of 4° Bé. and 10 litres of soap solution containing 55 about 0.6 kilogram of dry substance. All the impurities accumulate in this short liquor to a high concentration, and thus prevent the production of the new effect, and for this reason cloth which has been so treated does not show a capacity for repelling water even after it has been rinsed. 60

It is true that fine combed wool yarns are (before dyeing) treated a little more carefully with soap and soda, in order to remove the grease before dyeing, but even in this careful treatment the impure condition of the surface prevents the occurrence of the new effect, and further any indication of the new effect would be destroyed by subsequent dyeing. 65

The term wool in the sense of the present in- 70

vention comprises, in addition to sheep wool, animal hairs of all kinds and further so called artificial or old wool. The term textiles as used in the sense of the present invention includes 5 felt and similar materials made of wool.

I claim:

1. Process of rendering textiles of wool repellent to water, comprising thoroughly cleaning the textile of all impurities, subjecting it to 10 an additional treatment in a soap solution free of such impurities, and rinsing to remove the soap solution therefrom.

2. Process of rendering textiles of wool repellent to water, comprising thoroughly cleaning 15 the textile of all impurities, subjecting it to an additional treatment in a soap solution free of such impurities at a temperature of 25 to 50 degrees C., and rinsing to remove the soap solution therefrom.

20 3. Process of rendering textiles of wool repellent to water, comprising thoroughly cleaning the textile of all impurities, subjecting it to an additional treatment in a soap solution free of such impurities and containing from 1 to 4 grams of 25 soap per liter, and rinsing to remove the soap solution therefrom.

20 4. Process of rendering textiles of wool repellent to water, comprising thoroughly cleaning the textile of all impurities, subjecting it to an 30 additional treatment in a soap solution free of such impurities and containing from 1 to 4

grams of soap per liter and also containing sodium carbonate in quantity not exceeding 2 grams per liter for preventing acidity of the bath or material during the additional treatment, and rinsing to remove the soap solution 5 therefrom.

5. Process of rendering textiles of wool repellent to water, comprising thoroughly cleaning the textile of all impurities, subjecting it to an additional treatment in a soap solution free of such 10 impurities, rinsing to remove the soap solution therefrom, and repeating the treatment several times in pure soap solution and rinsing.

6. A process of rendering textiles of wool repellent to water, comprising subjecting the textile 15 to a cleaning and neutralizing treatment to remove all impurities and acidity, then subjecting it for 5 to 20 minutes to a treatment with an aqueous soap solution containing between 1 and 4 grams of soap per liter and itself free from 20 impurities at a temperature between 25 and 30 degrees C., and rinsing at a like temperature to remove the soap solution therefrom.

7. A water repellent wool textile having the fibers thereof prepared by thoroughly cleaning 25 the textile of all impurities, and thereafter subjecting it to an additional treatment in a soap solution free of such impurities and finally rinsing to remove the soap solution therefrom.

30

ALEXANDER NATHANSON.